

## UNITED STATES PATENT OFFICE

ALEXANDER MURRAY, OF ROCHESTER, NEW YORK, ASSIGNEE TO EASTMAN KODAK COMPANY, OF ROCHESTER, NEW YORK, A CORPORATION OF NEW YORK

## METAL CASTING FROM GELATIN RELIEFS

No Drawing.

Application filed May 11, 1932. Serial No. 610,745.

This invention relates to the making of metal casts from gelatin reliefs for the production of photomechanical printing plates. It is especially useful in metal casting from 5 gelatin molds in which there is comparatively deep detail of microscopic dimensions, such as the screen elements in photomechanical half-tone printing plate matrices.

It is particularly adapted to casting from 10 gelatin molds produced by the method described in the co-pending application, Serial No. 496,341, filed November 17, 1930 by M. Martinez. By that process, gelatin reliefs are developed by heat. When making metal 15 casts from such gelatin reliefs, the casting temperature cannot be much in excess of 200° C. and would preferably be about 150° C. Otherwise the texture of the surface of the gelatin is ruined and the resulting cast is very 20 poor or practically useless.

In casting from such molds which contain fine detail, such as fine half-tone dots, considerable difficulty is experienced. As it 25 covers the mold, the metal appears to trap a bubble of air in the depression. This bubble expands with the heat, producing a crater in the casting instead of a projecting point. The use of graphite and other powders, 30 greases, oils and other cushioning films is of no value. The same is true of lacquers, shellac, asphaltum resins, etc.

While soldering fluxes are common knowledge which contain organic acids such as 35 rosin (abietic acid), oleic acid, lactic acid and organic solvents such as lard oil, tallow, glycerin, etc., such fluxes are of no value as anti-gas trapping compounds in the method 40 of casting under consideration. The problems in the cases where fluxes are of value and in the present process do not appear to 45 be analogous even though the removal of metal oxides may be a mutually essential step.

I have found that satisfactory casts may be 50 obtained from gelatin molds such as that described by Martinez if the surface of the mold is coated before casting with a very thin layer of certain organic liquids. It is sufficient to rub the surface with a liquid of the 55 type described, removing any excess of liq-

uid by fairly vigorous means. If the temperature of the casting metal is not too high, a quite sharp cast can then be obtained.

The following formula is a typical and satisfactory example of a low melting point alloy in parts by weight:

|               |        |
|---------------|--------|
| Antimony----- | 1.34   |
| Lead -----    | 28.58  |
| Tin -----     | 16.52  |
| Bismuth ----- | 56.56  |
|               | 103.00 |

Melting point approximately 100° C.

After development of the relief, as for example, by the Martinez process, the surface of the relief is treated or coated with certain non-aqueous liquids which appear to have a specific tendency to prevent the trapping of gas in the depressions. It is possible that this is brought about at least partially by the tendency of these substances to dissolve the oxides of the alloy metals. As the metal flows onto the matrix, it probably accumulates a very thin film of oxides on its outer surfaces. This thin film or skin of oxide may then act to prevent the smooth flow of the casting metal into a very small, sharp depression.

In general, these liquids are organic liquids containing no water, they have a boiling point above the temperature of casting and they dissolve the oxides of the alloy metal. In certain cases, they appear to act more satisfactorily if they contain an aromatic carboxylic acid. Typical liquids which are especially useful are:

|                      |    |
|----------------------|----|
| Iso-amyl phthalate   | 89 |
| Anisaldehyde         | 90 |
| Cinnamaldehyde       | 90 |
| Quinoline            | 90 |
| n-butyl phthalate    | 93 |
| Decahydronaphthalene | 93 |

Suitable aromatic carboxylic acids which may be combined with these substances are anisic acid, cinnamic acid, phthalic acid and salicylic acid.

*Example I*

One of the most satisfactory of these substances is iso-amyl phthalate. In using this

substance, a small piece of cotton is moistened with iso-amyl phthalate and the surface of the mold is thoroughly wiped with it. Any excess of the liquid is carefully rubbed off with another piece of cotton. The mold is then ready for casting which may be done in a special frame under pressure. While if desired a number of casts may be made without re-treating the surface, it is best if other casts are to be made to rub the surface of the mold each time with the iso-amyl phthalate.

*Example II*

13 The saturated solution of anisic acid in anisaldehyde is also very satisfactory. The application of anisaldehyde to a gelatin relief requires a special technique because this liquid does not wet the untreated surface. 14 This, however, is easily overcome by first rubbing the surface thoroughly before development with aluminum bronze powder or graphite. The excess of powder is removed by wiping. After the relief has been obtained 15 by heat development, it is washed with a solution of anisic acid and anisaldehyde and the excess removed by thoroughly wiping with absorbent material so that only a minute quantity remains on the surface. Casts can 16 now be made with fusible alloys at, say 150° C. and the metal will properly fill detail of any character met with on a half-tone screen matrix.

*Example III*

17 The following solution is used:

|                   | Grams |
|-------------------|-------|
| n-butyl phthalate | 90    |
| Salicylic acid    | 10    |

18 This solution wets the surface of the relief without prior treatment. It is preferably applied after development of the relief just before casting. All excess is wiped away from the surface.

*Example IV*

|               | Grams |
|---------------|-------|
| Quinoline     | 18    |
| Cinnamic acid | 2     |
| Benzene       | 80    |

19 This solution can be applied more freely because it is diluted with benzene. When the benzene has evaporated, the remaining material can be wiped down as before.

*Example V*

|                    | Grams |
|--------------------|-------|
| Iso-propyl lactate | 95    |
| Phthalic acid      | 5     |

This liquid again may be used by merely applying, as described, and thoroughly wiping off any excess.

I consider as included in my invention all 70 modifications and equivalents coming within the scope of the appended claims.

What I claim is:

1. In the process of making a cast with an 75 easily fusible alloy from a gelatin mold in which there is fine detail, the step which comprises coating the said mold before casting with a very thin layer containing an organic liquid selected from the group consisting of iso-amyl-phthalate, n-butyl phthalate, quinoline, iso-propyl lactate, anisaldehyde, cinnamaldehyde, and decahydronaphthalene.

2. In the process of making a cast with an 80 easily fusible alloy from a gelatin mold in which there is fine detail, the step which comprises coating the said mold before casting with a very thin layer containing an aromatic carboxylic acid and an organic liquid selected from the group consisting of iso-amyl-phthalate, n-butyl phthalate, quinoline, 85 iso-propyl lactate, anisaldehyde, cinnamaldehyde, and decahydronaphthalene.

3. In the process of making a cast with an 90 easily fusible alloy from a gelatin mold in which there is fine detail, the step which comprises coating the said mold before casting with a very thin layer containing iso-amyl-phthalate.

4. In the process of making a cast with an 95 easily fusible alloy from a gelatin mold in which there is fine detail, the step which comprises coating the said mold before casting with a very thin layer containing anisaldehyde.

5. In the process of making a cast with an 100 easily fusible alloy from a gelatin mold in which there is fine detail, the step which comprises coating the said mold before casting with a very thin layer containing anisic acid and anisaldehyde.

6. In the process of making a cast with an 105 easily fusible alloy from a gelatin mold in which there is fine detail, the step which comprises coating the said mold before casting with a very thin layer containing an aromatic carboxylic acid and n-butyl phthalate.

Signed at Rochester, New York, this 5th day of May 1932.

ALEXANDER MURRAY.